

(No Model.)

W. HAINSWORTH.  
MAKING STEEL CASTINGS.

No. 284,004.

Patented Aug. 28, 1883.



Witnesses.  
C. Clarke  
R. H. Whartsey

Inventor. William Hainsworth  
By Attorney George A. Christy

# UNITED STATES PATENT OFFICE.

WILLIAM HAINSWORTH, OF PITTSBURG, PENNSYLVANIA.

## MAKING STEEL CASTINGS.

SPECIFICATION forming part of Letters Patent No. 284,004, dated August 28, 1883.

Application filed February 26, 1883. (No model.)

To all whom it may concern:

Be it known that I, WILLIAM HAINSWORTH, a citizen of the United States, residing at Pittsburgh, county of Allegheny, State of Pennsylvania, have invented or discovered a new and useful Improvement in Making Steel Castings; and I do hereby declare the following to be a full, clear, concise, and exact description thereof, reference being had to the accompanying drawing, making a part of this specification, which represents a portion of a mold for casting steel rolls, the same being illustrative of my invention.

My invention relates to the art of making steel castings for rolls, shafts, and similar articles; and, in general terms, it consists in introducing a metal chill or heat-absorbing core in the center or axis of the body of metal filling the mold-cavity, in order to hasten the cooling and crystallization of the inner mass of metal, and also to counteract rapid and unequal contraction of the outer surface by expansion within, thereby preventing unsoundness and distortion by shrinkage, as hereinafter more fully described and claimed.

I have illustrated my invention applied to the casting of a steel roll; but it may be applied to other forms of steel castings in substantially the same way.

In casting steel rolls it is customary to make use of a sand-mold—such, for example, as is represented in part in the drawing and lettered A—having therein a mold-cavity corresponding to the form of roll C to be produced, which latter consists of a body portion, c, of cylindrical form, shoulders c', of less diameter than the body, and necks c'', of still less diameter than the shoulders.

The sprue or pouring-hole of the mold-cavity is usually made at one end communicating with the neck, and the opening thus made is enlarged somewhat, as at D, to hold a supply of metal in excess of that required to fill the mold-cavity proper. This cavity D, or the supply of metal therein, is technically known as the "sinker-head," and it is designed to afford a supply of metal to fill up any space or opening which might otherwise be formed by shrinkage of the metal in cooling. With castings of moderate sizes this method of preventing shrinkage usually accomplishes the desired

result; but in large or heavy castings, owing largely to the slow rate of cooling of the interior body, compared with the exterior surface, such provision often fails of securing the desired soundness of body or mass and perfectness of form. In roll-casting, this difficulty is aggravated by the special form of the article. The neck, being smaller than the body portion, cools and crystallizes first, thus arresting the supply of metal from the sinker-head. Consequently further cooling of the body after the neck is closed results in more or less contraction, unsoundness, and distortion, such distortion usually taking place at or near the angle of the upper end of the body and in the upper shoulder, as indicated by dotted lines s. In other forms of heavy castings—such, for example, as are made for subsequent working and reduction into steel shafts for use in heavy machinery—there is great danger of unsoundness, hollow centers, and ruptures, owing to rapid cooling on the exterior and slow protracted cooling in the inner mass of metal. The loss ordinarily sustained in heavy steel castings from difficulties of this nature is considerable, and largely increases both the risks and expense of manufacture.

In applying my invention to roll-casting, molten steel is poured into the mold A, filling its cavity, and also partially filling the sinker-head cavity, D. I then insert into the central body of metal a solid and preferably cold body of steel, E, having length a little less than the body c of the casting, and thickness, say, about one-third of the full diameter of such body, or less than the diameter of the neck c''.

A core, E, of iron, may be employed instead of steel. I prefer steel, however, and that of the same or approximately the same grade as the molten metal, in order to avoid chemical action, which is liable to arise when different grades of metal are employed, with attendant liberation of gases and formation of blow-holes. This trouble may be obviated in great measure, however, if iron be used, by coating it with plumbago or other similar carbonaceous material. This core E is supported and manipulated by means of a comparatively small rod, e, welded or otherwise secured thereto, and having an eye or hook, e', in its free end, in which a crane-chain is secured to manipulate

the core by power-lift. This rod *e* may be of iron or steel. For convenience in welding it to the core I prefer to employ iron, and to coat it with plumbago or equivalent material, to prevent direct contact of molten steel therewith. This body of cold metal *E*, inserted within the central mass of molten metal, will quickly absorb or take up a large amount of heat. In this way the whole mass of metal in the body part *c* of the roll may be cooled substantially in the same time as the metal in the neck *c'*. Consequently metal in the sinker-head will be free to settle into the body part of the cavity until the major part of contraction by cooling has taken place, thus preventing contraction in the upper end of the roll to any injurious extent.

In order to secure the best results, the rod *e* should, if the pouring end of the casting is smaller than the body below, be comparatively light, in order to produce but little chilling effect upon the metal in such smaller portion; also, the core *E* should be somewhat shorter than the body part *c* of the roll; but these proportions may be varied considerably, depending upon the particular form of casting. For example, if the casting be of uniform size throughout, as in casting ingots for shafting, the core may also be of similar form. Another important function of the core in this improvement is to occupy the center of the casting with solid metal, which is expanded by heat as the molten metal contracts, thereby counteracting the contracting tendency of the exterior. Owing to rapid absorption of heat by the core, the greater part of its expansion takes place soon after its immersion in the molten metal; but the greatest danger to the casting occurs some time after pouring, or after the metal of the surface has become crystallized.

By inserting the core after pouring I am enabled to introduce it at such time as to derive the most benefit from its expansion, at the same time keeping in view the beneficial results of uniform crystallization throughout the mass of the casting. If, as practiced heretofore, the core is placed in the mold before pouring, its expansion by heat takes place too soon to be of material benefit, and also danger is incurred of causing the molten metal to spatter or bubble. If the core is inserted after pouring and then withdrawn, as practiced in making tubular castings, it must be withdrawn so soon, in order to prevent fusion, that little ex-

pansion takes place, and little or none of the benefits above described are secured; but by inserting the core after pouring and permitting it to remain and fuse with the molten metal, as above described, solid metal is insured at the core or center, and also the surface-strain caused by rapid cooling on the exterior without corresponding cooling and contraction of the interior is to a great degree prevented. The size of core to be employed in each case will be determined by the size and form of the casting, reference being had to securing a fused union between the core and molten metal, and to this end the core should not be so large as to chill the metal below a degree which will admit of such fusion before or when uniform temperature is secured at and near the surface of the core. The skilled workman can readily make the requisite provision in this respect, knowing the results which it is desired to attain.

This improved method of casting, whether of rolls or other products, can be applied to advantage either with or without a chill surrounding the mold-cavity.

I claim as my invention—

1. The method herein described of making solid steel castings, consisting in filling the mold-cavity with molten steel, and subsequently inserting in the axis or central mass of fluid metal within the mold a solid metallic core, permitting such core to remain and fuse with the previously-poured metal, substantially as and for the purposes set forth.

2. The method herein described of casting solid steel rolls having necks of less diameter than the body, consisting in pouring the molten steel into the mold-cavity through the upper neck, and subsequently lowering a solid steel core through the neck or pouring-opening into the axial center of the body part of the mold, and permitting such core to remain therein, the solid and fluid steel being together sufficient in amount to fill the mold-cavity and fill or partially fill the sinker-head, substantially as described.

In testimony whereof I have hereunto set my hand.

WILLIAM HAINSWORTH.

Witnesses:

OLIVER FULTON,  
C. S. PARKER.